

Oct. 22, 1929.

F. S. McCULLOUGH

1,733,082

METHOD OF AND APPARATUS FOR COATING CATHODES

Filed May 14, 1925



INVENTOR.  
Frederick S. McCullough  
BY *O.M. Clarke*  
ATTORNEY.

## UNITED STATES PATENT OFFICE

FREDERICK S. McCULLOUGH, OF WILKINSBURG, PENNSYLVANIA

## METHOD OF AND APPARATUS FOR COATING CATHODES

Application filed May 14, 1925. Serial No. 30,181.

The present invention relates to the coating of cathode structures for use in electron tubes.

In certain types of thermionic tubes, the cathode is in the form of a metal sleeve which surrounds and is fitted on a suitable heating element. In order to get the best results, it is desirable to coat these sleeves with an emitting substance. As such emitting substance 10 has to be baked onto the metal of the cathode, and as metals desirable for this purpose are of a readily oxidizable nature, and as the oxidation of the metal of the cathode between the coating and the body of the cathode seriously 15 impairs the cathode, care must be taken to prevent such oxidation.

The present invention has for its object to provide a method of and apparatus for the convenient, rapid, and efficient coating of such 20 tubular cathodes.

The nature of the invention may be best understood by reference to the accompanying drawings, in which:

Fig. 1 represents a vertical section through 25 an apparatus for practicing the invention;

Fig. 2 is a plan view of a part of the dipping rack;

Fig. 3 is a broken side view of the dipping 30 rack, showing cathodes in place thereon;

Fig. 4 is a detail view of one of the cathodes.

As the nature of the invention may be best understood by understanding the structure of the cathode, reference may be first made to Fig. 4. In this figure, A is a metal sleeve, 35 preferably continuously cylindrical and preferably formed of thin sheet metal of a suitable nature. Nickel is preferably used as the metal for the sleeve. Welded or otherwise secured to the sleeve is a lead wire or stem B 40 of a suitable nature.

In practicing the invention, the sleeves A are first preferably treated to drive out the contained gases, particularly air. This may be done by baking in a suitable apparatus, 45 either in a vacuum or in a suitable atmosphere of inert gas, such as hydrogen. When the air is driven out of the metal, it is not rapidly absorbed again, and the sleeves may be exposed to air for a considerable time without 50 injury.

After being so treated, the stems or wires B are attached. The cathodes are then threaded or arranged end-to-end on wires 5 having head portions 6 on their upper ends. These wires form a removable part of a dipping 55 rack. This dipping rack has a central rod or stem 7 having two spaced apart disks 8 and 9 thereon, the lower disk 9 being at or near the bottom of the stem.

These disks are of the form shown in Fig. 60 2, having radial notches 10 therein, which are preferably enlarged at their inner ends. The tops of the wires 5 slip into the notches of the upper disk, while the heads 6 thereof prevent them from slipping down. The lower ends 65 of the wires are received in the notches of the lower disk, retaining the cathodes on the wires and holding the lower ends of the wires in spaced relation. Fig. 3 clearly illustrates the construction of the rack and the manner of 70 placing the cathodes thereon.

When the desired number of cathodes have been arranged on the rack, they may be coated. To this end, a special apparatus such as that 75 shown in Fig. 1 has been designed.

The apparatus includes an upper casing 11 of glass or other suitable material, open at its top and bottom. A layer of insulating material may surround the lower portion of the casing, and within this layer of insulating 80 material is a coil 12 in circuit with a suitable source 13 of high frequency current. The part of the casing surrounded by the coil forms the baking or heating chamber, while the portion 11<sup>a</sup> extending above the heating 85 chamber is a cooling chamber. Fitted into the lower end of the outer casing, and preferably detachable therefrom, is a cylindrical container 14. This container is of sufficient depth to contain sufficient liquid to enable 90 the sleeve carrying portion of the dipping rack to be immersed. At the bottom of the receptacle is an inlet pipe 15.

The receptacle is filled to a sufficient depth with a solution or thin paste containing the 95 coating compound, such as an alkaline earth carbonate and water. The carbonate is finely divided or comminuted so as to readily stay in suspension in the liquid. This may be kept in a constant state of agitation by 100

the introduction of an inert gas, such as carbon dioxide through the inlet pipe 15. This gas not only keeps the mixture or solution agitated, but fills the interior of the upper casing 11 and 11<sup>a</sup>.

5 The rack charged with cathodes is lowered into the apparatus as shown in Fig. 1, until the rack is immersed in the coating mixture in the receptacle. The rack is then raised 10 into the upper casing and the coil 12 is energized.

15 The oscillating field set up by the coils effects a heating of the cathodes and bakes the coating material thereon. Care must taken, however, to so control the baking or 20 heat treatment that the temperature thereof does not cause the oxidation of the nickel or metal of the cathode. After the coating has been baked on, the rack is raised out of the furnace through the upper extension 11<sup>a</sup>, where they cool in an atmosphere of CO<sub>2</sub> gas before being taken out into the air.

25 Obviously any suitable heating means could be substituted for the radio-frequency coil, although the temperature can be quite accurately controlled with a radio frequency coil.

30 I have illustrated a preferred form of my invention, but it will be understood that various changes are contemplated under the scope and spirit of the invention.

I claim as my invention:

35 1. The method of coating oxidizable cathode bodies which consists in immersing the bodies in a coating bath, and immediately baking the adherent coating in an atmosphere of inert gas, and then cooling said cathode in said inert gas.

40 2. The method of coating oxidizable metal cathodes which consists in immersing the cathodes into a coating paste, raising the cathodes out of the paste into a heating chamber and baking on the adherent coating in an atmosphere of inert gas, and cooling 45 the cathodes in an atmosphere of inert gas.

45 3. The method of coating oxidizable metal cathodes which consists in immersing the cathodes in a coating paste, raising the cathodes vertically into a heating chamber and baking on the adhering coating while in an atmosphere of carbon dioxide gas, and then raising the cathodes through a chamber containing an atmosphere of carbon dioxide.

55 4. The method of coating metallic cathode bodies which consists in driving out absorbed air from the bodies, dipping the bodies in a coating bath, and baking the adhering coating in an atmosphere of inert gas, and then 60 raising the cathode into a chamber containing the inert gas.

55 5. An apparatus for coating cathodes comprising a baking furnace, a dipping vessel at 65 bottom of the furnace and forming a continuation thereof, and a cooling chamber at

the top of the furnace and forming a continuation thereof.

6. An apparatus for the coating of cathodes comprising an elongated vertical furnace structure provided with a heating coil 70 on the outside thereof, an elongated receptacle at the bottom thereof, and an elongated vertical cooling chamber at the top thereof and forming a continuation thereof.

7. An apparatus for the coating of cathodes comprising an elongated vertical furnace having a vertical chamber therein, an elongated receptacle containing a coating bath removably connected with the bottom thereof and forming an extension thereof, 80 and means connected to said receptacle for introducing gas into said receptacle near the lower end thereof.

8. An apparatus for coating cathodes comprising a baking furnace, a dipping vessel at the bottom of the furnace, and forming a continuation thereof, a cooling chamber at the top of the furnace and forming a continuation thereof, and means connected to 90 said dipping vessel for supplying carbon dioxide gas to the lower end of the dipping vessel, said apparatus having an opening at its top.

In testimony whereof I hereunto affix my signature.

FREDERICK S. McCULLOUGH.

100

105

110

115

120

125

130